

# UNITED STATES PATENT OFFICE.

JOSEPH YATES, OF MOTT HAVEN, NEW YORK.

## ELECTRO-DEPOSITION OF NICKEL.

SPECIFICATION forming part of Letters Patent No. 224,263, dated February 3, 1880.

Application filed April 17, 1879.

*To all whom it may concern:*

Be it known that I, JOSEPH YATES, of Mott Haven, in the city, county, and State of New York, have invented or discovered certain new and useful Improvements in the Electro-Deposition of Nickel, of which the following is a specification.

It is well known that nickel has been found to be one of the most difficult metals to deposit successfully by electrolysis, and that heretofore the solutions used for nickel-plating have been of a compound nature, in most, if not all cases, consisting of double salts, such as the double sulphate of nickel and ammonia, or chloride of nickel and ammonia. Indeed, it has been heretofore held as impracticable to nickel-plate with a single salt. I have succeeded, however, in producing deposits of nickel from a solution of a simple single salt which presents advantages which I believe are unique and superior to what has heretofore been effected; and the essential feature of my invention or discovery may be stated to consist in electroplating with nickel by means of a solution of the acetate of nickel.

For the purposes of my invention the acetate of nickel may be prepared in any of the ways known to chemists, and which do not here require description. It is, of course, preferable that the salt be as pure as possible; but the qualities of a solution of this salt for plating are such that absolute purity is not essential, and its preparation does not, therefore, require such expensive care as is the case with the compounds heretofore used for this purpose.

For the purpose of plating, the acetate of nickel is dissolved in clear water, the solution being made of a strength preferably from  $8^{\circ}$  to  $10^{\circ}$  Baumé; but it may be weaker. This solution is used in the plating apparatus in the same manner as the solutions employed heretofore, the battery being connected therewith, and a nickel anode being employed in the usual manner, as is well understood by electroplaters. This solution, however, has the great advantage that it contains a much larger proportion of metal than the nickel-salt solutions heretofore used, and is hence a good conductor of the current, and, moreover, is easily decomposed thereby, so that a much

weaker current suffices to produce a successful deposit of the metal. Furthermore, as the solution is of a simple nature, being a single salt of a weak organic acid, it is not subject to those irregular decompositions which render the management of the usual double salt solution so difficult and require such careful regulation of the current and the avoidance of any slight acid or alkaline impurity. Thus it is well known to platers that those compound solutions containing salts of strong acids or strongly corrosive substances, such as chlorine and sulphur, are subject, under any irregular conditions, to changes or decompositions which cause corrosions of the article being plated, commonly termed "burning." The simple solution of acetate of nickel, however, which I employ is found to be quite free of any such tendency, which is ascribable, it is believed, to the weak nature of its acid, its large amount of metal, and the simple nature of the salt, it being an obvious principle that the simpler are the conditions the less liability is there to confusion or irregularity in the action.

A most important advantage of this acetate-of-nickel solution yet to be mentioned is that by it the plater is enabled to plate with nickel directly on metal, which it has been heretofore impracticable or quite difficult to nickel-plate without a previous coating of copper. Thus by means of this solution I am enabled to plate steel and cast or wrought iron directly with a coating of nickel of sufficient thickness for protection, and of a perfectly adhering, close, and tough quality, which is believed to be a result quite unique and of great importance in the arts.

The previous or existing modes of nickel-plating, as is well known, are not adapted for common or cheap articles of iron or steel, as in most all cases a previous coating of copper is required, and the expense of such double coating of copper and nickel is found to be too great to be adapted to articles for general sale, while, furthermore, unless the operation is carefully conducted, the adhesion of the deposit is not good. My improvement in the art, however, enables common articles of hardware in cast or wrought iron or steel to be plated directly with a lasting and ornamental

coating of nickel, which greatly enhances their salable and wearing qualities, and but slightly increases their cost—a result long sought for, but not heretofore attained—while the adhesion of the nickel directly to the iron is actually found to be superior to the adhesion of copper in copper-plating, which constitutes, it is believed, an important advance in the art.

The qualities of the deposit produced from this solution of acetate of nickel is found to be excellent, being smooth, brilliant, and tough, and free of any granular or scaly tendency.

Most all metals can be directly plated from this solution, the most difficult metals to plate being the soft poorly-conducting metals; but among these zinc—the most commonly used—can, with care, be well plated.

I may mention that another salt may sometimes be combined with the acetate of nickel, such as acetate of ammonia; but I prefer to use the acetate of nickel alone. It will also be understood that my invention is, of course, applicable to producing deposits of nickel for the purpose of electrotyping as well as for ordinary plating, or for any other electro-deposition of nickel.

What I claim as my invention is—

The electro-deposition of nickel by means of a solution of acetate of nickel, substantially as herein set forth.

JOSEPH YATES.

Witnesses:

JOHN E. GAVIN,  
CHAS. M. HIGGINS.